# EUROPEAN PATENT SPECIFICATION

(11) **EP 1 214 200 B1**
(45) Date of publication and mention of the grant of the patent: **24.03.2004**
(21) Application number: 00904504.8
(22) Date of filing: 21.01.2000
(51) Int. Cl.: B41M 5/00

(54) **INK-JET RECEPTOR SHEET, AND METHOD OF MANUFACTURING AND USING THE SHEET**
TINTENSTRAHLEMPFANGSBLATT, UND VERFAHREN ZUR HERSTELLUNG UND VERWENDUNG DES BLATTS
FEUILLE DE RECEPTION DE JET D'ENCRE ET SON PROCEDE DE FABRICATION

(30) Priority: 12.08.1999 US 372582
(43) Date of publication of application: 19.06.2002
(73) Proprietor: Kodak Polychrome Graphics LLC, Norwalk, Connecticut 06851 (US)
(72) Inventor: YARMEY, Susan, K., Saint Paul, MN 55164-0898 (US); STEINER, Michael, L., Saint Paul, MN 55164-0898 (US)
(74) Representative: VOSSIUS & PARTNER
(86) International application number: PCT/US2000/001636
(87) International publication number: WO 2001/012446

(56) References cited:
- EP-A- 0 199 874
- EP-A- 0 736 392
- WO-A-95/28285
- WO-A-99/06219
- GB-A- 2 147 003
- PATENT ABSTRACTS OF JAPAN vol. 1996, no. 6, 28 June 1996 (1996-06-28) & JP 08 034160 A (FUJI PHOTO FILM COMPANY LIMITED), 6 February 1996 (1996-02-06)

## Description

The invention broadly relates to image receiving elements and methods of manufacturing and using such elements. More specifically, the invention relates to inkjet receptors, also known as inkjet recording sheets, and methods of manufacturing and using such elements.

Ink jet printing is a printing technique in which images (*e*.*g*., graphs, pictures, symbols, text, etc.) are produced by the ejection of uniformly shaped droplets of ink onto the receptor surface of a recording sheet. This printing technique is widely used in the personal and small office markets. Other applications include low end proofing, and medical referral markets.

The maximum image resolution and throughput of an ink jet printer are primarily determined by the size of the jetted drop and the rate of drop ejection. Several factors limit inkjet printers from attaining the maximum image resolution capable of being achieved by the printer. One of these limiting factors is the nature of the recording sheet receiving the jetted drops.

Investigators have found image quality to be directly related to the ink absorption and dye adsorption rate of the receptor surface, with image quality increasing with an increase in absorption and adsorption rates. As a general matter, investigators have found that when the ink droplets are not absorbed quickly enough, the ink tends to spread and interact with neighboring droplets of ink, resulting in such defects as feathering, pooling, or bleeding. Investigators have also found that when the ink is not adsorbed quickly enough, the ink tends to bleed through the receptor and possess reduced resolution, reduced water fastness, and reduced smudge resistance. Such problems are exacerbated as the droplet ejection frequency is increased for purposes of increasing throughput.

Ink receptor surfaces can be divided into two basic types: continuous phase systems and discontinuous phase systems. Continuous phase systems generally function by swelling to absorb water or ink deposited onto the receptor surface, with the rate of absorption determined by the chemical nature of the polymer used in the system. Typical polymers used in continuous phase systems include gelatins, polyvinyl alcohol and cellulose. Exemplary continuous phase systems are discussed in United States Patents Nos. 3,889,270, 4,503,111, and 5,141,599.

While generally effective as an ink jet receptor surface, most polymeric continuous phase systems are water soluble, thereby reducing the waterfastness of the receptor, Some polymeric continuous phase systems have overcome the waterfastness issue by mixing an insoluble cross-linked polymer into the system (*e*.*g*., forming a semi-interpenetrating network as described in United States Patents Nos. 5,342,688 and 5,389,723). However, the introduction of an insoluble cross-linked polymer into the system intrinsically reduces the absorption rate of the system.

Discontinuous phase systems function by providing pores within the receptor surface capable of absorbing ink by capillary forces. Discontinuous phase systems are generally preferred over continuous phase systems as they absorb ink considerably faster than continuous phase systems.

Discontinuous phase systems are divided into two basic types. A first type of a discontinuous phase system, known as a "porous discontinuous phase system", utilizes micron sized porous pigment particles in the recording layer for purposes of absorbing ink jetted onto the recording layer into the particles through a multitude of tiny interconnected pores in each particle. Ink recording sheets having a porous, discontinuous phase system recording layer are disclosed in United States Patent Nos. 5,165,973; 5,270,103; 5,397,619; and 5,478,631, and International Published Application WO 97 01448.

A second alternative type of discontinuous phase system, known as a "nonporous discontinuous phase system" utilizes nonporous pigment particles held together by a polymeric binder in such a manner that interstitial voids are created between the pigment particles capable of absorbing ink jetted onto the receptor surface.

Ink jet recording sheets with a recording layer of the porous discontinuous phase system type generally provide good ink absorptivity and superior ink capacity, in exchange for some loss in the glossy appearance of the recording sheet. Alternatively, ink jet recording sheets with a recording layer of the nonporous discontinuous phase system type provide superior ink absorptivity and a glossy appearance in exchange for a limited ink capacity due to practical limitations upon the thickness of the coating.

Discontinuous phase system receptor surfaces often incorporate a mordant or dye fixing agent for purposes of binding the dye molecules adsorbed within the pores of the receptor surface. A number of different types of mordants have been used, including neutral silane coupling agents, such as disclosed in JP 8164667 (polyalkylene oxide silane), JP 3218887 (silicon compounds), JP 62178384 (silane coupling agents) and JP 60224580 (silane coupling agents with chloro, amino, aminoethyl or vinyl functionality); and monomers, oligomers and polymers of primary, secondary and tertiary amines and quaternary ammonium salts, such as disclosed in United States Patents Nos. 5,302,437 and 5,750,200.

WO-A-99 06219 discloses an ink jet recording sheet wherein the surface of the sheet is coated with an ink receptive layer of an aqueous sizing medium containing a divalent metal salt such as calcium chloride and magnesium chloride. The sizing medium may include other conventional additives such as carrier agents, fillers, optical brightening agents, defoamers and biocides.

WO-A-95 28285 discloses an ink jet recording sheet wherein the surface of the sheet is coated with an ink receptive layer containing a trivalent salt or complex of a Group IIb metal, such as lanthanum. The salts can also be used in the form of their double salts containing Ca, Mg, Ba, Na, K or the like. The ink receptive layer preferably includes a film forming hydrophilic polymeric material.

GB-A-2 147 003 discloses an ink jet recording sheet wherein the surface of the sheet is coated with an ink receptive layer containing a binder, a pigment, a watersoluble salt with a valency of 2 to 4, and a cationic organic material.

EP-A-0 736 392 discloses an ink jet recording sheet wherein the surface of the sheet is coated with an ink receptive layer containing an alumina hydrate having a boehmite structure and a binder. The ink receptive layer may also include metal oxides, polyvalent metal salts, and cationic organic substances. The dry ink receptive layer may be treated with a metal alkoxide or other material capable of crosslinking a hydroxyl group to the ink receptive layer.

EP-A-0 199 874 discloses an ink jet recording sheet wherein the surface of the sheet is coated with an ink receptive layer containing polyethylene oxide and a white filler. The ink receptive layer preferably also includes a cationic resin and/or polyvalent metal salt. The ink receptive layer may also include a resin.

While neutral silane coupling agents, cationic monomeric, oligomeric and polymeric amines, and quaternary ammonium salts are generally effective for providing an acceptable rate of adsorption of dye to a receptor surface, a substantial need continues to exist for an ink receptor surface capable of providing a superior dye adsorption rate while maintaining dye adsorption capacity, bonding strength of the dye to the surface of the receptor layer, ink absorption rate and ink absorption capacity.

A first aspect of the invention is an ink jet recording sheet providing a superior adsorption rate of dye by the receptor layer while maintaining dye adsorption capacity, bonding strength of the dye to the surface of the receptor layer, ink absorption rate and ink absorption capacity, comprising a receptor layer of a binder, pigment particles, an electrolyte, and a cationic organosilane coupling agent.

A second aspect of the invention is a method of making an inkjet recording sheet comprising (1) coating a layer of a recording composition on a major surface of a substrate wherein the recording composition is a dispersion containing at least (i) a binder, (ii) pigment particles, (iii) an electrolyte and (iv) a cationic organosilane coupling agent and (2) drying the recording layer.

A third aspect of the invention is a method of using an ink jet recording sheet comprising (1) obtaining a substrate having a layer of a recording composition on at least one of the major surfaces of the substrate, wherein the recording composition is a dispersion comprising at least (i) a binder, (ii) pigment particles, (iii) an electrolyte and (iv) a cationic organosilane coupling agent and (2) jetting inkjet printing ink upon the major surface of the substrate coated with the recording composition so as to produce an image upon the sheet.

### BRIEF DESCRIPTION OF THE DRAWINGS

Figure 1 is an enlarged side view of one embodiment of the invention.

### Nomenclature

- **10**: Ink Jet Recording Sheet
- **20**: Substrate
- **30**: Subbing Layer
- **40**: Recording Layer
- **50**: Anti-curling Layer

### Definitions

As utilized herein, including the claims, the term "*thickness*", when used in connection with the recording layer, means the thickness of the recording layer on a dry basis.

As utilized herein, including the claims, "*wt%*" is based upon the solids content of the composition (*i*.*e*., calculated on a dry basis).

### Construction

The discontinuous ink jet recording sheet **10** includes a coating of a discontinuous recording layer **40** on a suitable substrate **20**, wherein the recording layer **40** is capable of quickly adsorbing dye while maintaining dye adsorption capacity, bonding strength of the dye to the surface of the receptor layer, ink absorption rate and ink absorption capacity.

### SUBSTRATE

The substrate **20** may be any of the typical materials used in the construction of ink jet recording sheets capable of providing the necessary visual appearance and structural support for the recording layer(s) **40**. Examples of suitable substrates include paper, cloth, polymers, metals, and glass. Thin flexible sheets are generally preferred, with paper being the substrate of choice when an opaque support is desired, and polymeric films used when a translucent or transparent appearance is desired. The thickness of the substrate **20** is preferably in the range of about 0.05 to 1.0 mm.

### SUBBING LAYER

The major surface of the substrate **20** to be coated with the recording layer **40** may optionally be treated with a subbing layer **30**, such as a primer or an antistatic layer, before the recording layer **40** is coated onto the substrate **20**.

### RECORDING LAYER

The recording layer **40** is comprised of pigment particles treated with an electrolyte and held together by a binder. The recording layer **40** should have a thickness of greater than about 30 µm in order to provide sufficient capacity. Recording layers **40** possessing an acceptable appearance can be formed up to a thickness of about 100 µm, with a thickness of between about 35 to 85 µm preferred.

### Pigment Particles

The recording layer **40** contains pigment particles of the type conventionally used in ink jet recording layers. The pigment particles may be porous or nonporous. Exemplary pigment particles include specifically, but not exclusively, (i) inorganic pigments such as alumina, aluminum hydroxide, aluminum oxide, aluminum silicate, barium sulfate, calcium carbonate, calcium silicate, calcium sulfate, kaolin, magnesium silicate, amorphous silica, colloidal silica, silicic acid, sodium silicate, talc, titania, titanium dioxide, zinc carbonate, and zinc oxide, and (ii) organic pigments such as styrene and acrylic plastic pigments, urea resin pigments, and melamine resin.

Pigment particles having an average particle size of less than about 500 nm are capable of producing a recording layer **40** having the desired appearance and performance. Pigment particles having an average particle size of between about 10 - 500 nm are generally preferred, with particles having an average particle size of between about 50 - 300 nm desired and particles having an average particle size of between about 50 - 100 nm favored.

The pigment particles can be of substantially any desired shape, with symmetrical particles, particularly spherical particles, generally preferred as they enhance the performance characteristics of the recording layer **40**.

### Binder

The pigment particles are held together by a binder. The binder is provided in an amount sufficient to hold the pigment particles together and provide an acceptable appearance. It is generally desired to limit the amount of binder so as to provide pores (i.e., interconnected interstitial voids) within the recording layer **40** for purposes of enhancing performance. Ink jetted onto the recording layer **40** will be absorbed into and stored within the pores (*i*.*e*., pores within the pigment particle or pores between the pigment particles) in the layer **40** through capillary action.

Substantially any of the conventional binders may be employed, including specifically, but not exclusively: starch derivatives such as oxidized starch, etherified starch and phosphate starch; cellulose derivatives such as carboxymethyl cellulose and hydroxymethyl cellulose; conjugated diene-type copolymer latexes such as styrene-butadiene and methyl methacrylate-butadiene copolymers; acrylic polymer resins and latexes such as polymers and copolymers of acrylic and methacrylic acid esters; vinyl-type polymer latexes such as ethylene-vinyl acetate copolymer; the aforementioned latexes modified to include a functional group such as a carboxyl group; aqueous adhesives such as melamine or urea resins; synthetic resins such as polyurethanes, unsaturated polyesters, vinyl chloride-vinyl acetate copolymer, polyvinyl butyral and alkyd resins; casein, gelatin, soybean protein, polyvinyl alcohol and derivatives thereof, polyvinyl pyrolidone, and maleic anhydride resins.

### Relative Concentrations of Pigment Particles and Binder

The amount of binder used in the recording layer **40** relative to the amount of pigment particles should be selected to balance the competing interests of integrity and wear resistance (enhanced by increased amounts of binder) with ink absorption rate and ink absorption capacity (enhanced by decreased amounts of binder). Hence, a careful consideration of binder concentration is important to create a suitable inkjet recording layer 40 having a proper balance of performance characteristics. As a general matter, a weight ratio of pigment to binder of about 1:2 to 20: 1, preferably about 2:1 to 10:1, provides acceptable balancing of the competing performance characteristics.

### Electrolyte

The recording layer **40** includes an electrolyte. As utilized herein, electrolyte means a substance effective as an ionic conductor when dissolved in a suitable solvent. In other words, the substance dissociates into anions (negatively charged particles) and cations (positively charges particles) when dissolved.

Suitable electrolytes includes specifically, but not exclusively, acids such as acetic, butyric, chloroacetic, lactic, and tartaric; inorganic salts such as sodium chloride, calcium chloride, ammonium sulfate, sodium sulfate, aluminum chloride, calcium sulfate, iron chloride, potassium chloride, potassium carbonate, lithium bromide and zinc sulfide.

The recording layer should include about 0.5 to 25 wt%, preferably about 1 to 15 wt%, electrolyte. Insufficient electrolyte does not produce a meaningful increase in the rate of dye adsorption while an excess of electrolyte tends to interfere with the other desired properties of the recording layer.

### Cationic Silane Coupling Agent

The recording layer includes a cationic organosilane coupling agent. Suitable cationic organosilane coupling agents include a first moiety (R') capable of dissociating in water to produce a positively charged group on the organosilane coupling agent, and a second moiety (R") effective for bonding to the pigment particles. When dissociated, the first moiety is effective for electrostatically attracting and forming an insoluble salt with dyes having an electron donating group (*e*.*g*., an -SO₃⁻) such as is present on many of the Azo, direct and acid dyes typical of inkjet inks.

Preferred cationic silane coupling agents possess the basic structure:

R'L SiR"₃

wherein: (i) R' is a quaternary ammonium group, (ii) L is a single bond or divalent linking group, and (iii) each R" is independently an alkoxy group.

A more preferred cationic organosilane coupling agent has the basic structure:

R'ₙ Si R"₍₄₋ₙ₎

wherein: (i) R' is -R³₃N⁺L- where L is a single bond or divalent linking group, and each R³ is independently hydrogen, alkyl, aryl or alkaryl with at least two R³ being alkyl, aryl or alkaryl, (ii) each R" is independently an alkoxy group; and (iii) n is 1 or 2.

Exemplary suitable cationic organosilane coupling agents include specifically, but not exclusively: N,N-didecyl-N-methyl-N-(3-trimethoxysilylpropyl) ammonium chloride, octadecyldimethyl (3-trimethoxysilylpropyl) ammonium chloride, N-trimethoxysilylpropyl-N,N,N-trimethylammonium chloride, tetradecyldimethyl (3-trimethoxysilylpropyl) ammonium chloride, N-trimethoxysilylethyl benzyl-N,N,N-trimethyl ammonium chloride, N-(trimethoxysilylpropyl) isothiouronium chloride, N-trimethoxysilylpropyl-N,N,N-tri-n-butyl ammonium chloride, N-trimethoxysilylpropyl-N,N,N-tri-n-butyl ammonium bromide, 3-[2-N-benzylaminoethylaminopropyl] trimethoxysilane hydrochloride, N-(3-trimethoxysilylpropyl)-N-methyl-N,N-diallyl ammonium chloride, and 3-N-styrylmethyl-2-aminoethylamino-propyltrimethoxysilane hydrochloride.

### Additives

Other typical additives such as dispersants, lubricants, surfactants, plasticizers, antistatic agents, pH adjusters, buffers, coating aids, matting agents, particulates for managing mechanical processing of the ink jet recording sheet, antifoaming agents, foam suppressants, water-proofing agent, hardeners, colorants, viscosity modifiers, preservatives, ultraviolet absorbent, antioxidants, antiseptics, mildewproofing agents, and the like may optionally be incorporated into the inkjet recording layer as desired.

### ANTI-CURLING LAYER

An anti-curl layer **50** may optionally be coated on the back side of the substrate **20**.

### Method of Manufacture

### BLENDING OF CONSTITUENTS

The constituents of the recording layer may be blended together by substantially any convenient method. Exemplary procedures include, (i) sequentially charging pigment, electrolyte and binder into a sufficient quantity of solvent (preferably water) under constant agitation, (ii) simultaneously charging the pigment, electrolyte and binder with sufficient solvent into a suitable mixer, and (iii) dispersing the pigment in water, adding the electrolyte to the aqueous dispersion of pigment, and then adding the electrolyte-containing aqueous dispersion of pigment into an aqueous dispersion of the binder.

### COATING AND DRYING OF RECORDING LAYER

The recording layer **40** may be coated by any of the conventional techniques for coating such materials, including specifically, but not exclusively, extrusion coating, direct and indirect gravure coating, knife coating, Mayer rod coating, roll coating, etc.

Similarly, the coated recording layer **40** may be dried by any of the conventional techniques for drying such coated recording layers.

### OPTIONAL PROCESSING

The recording layer **40** can be calendered to improve gloss, with the calendar rolls heated or unheated and rotating concurrent or countercurrent with respect to the movement of the ink jet recording sheet **10**.

### EXPERIMENTAL

### Glossary

| | |
|---|---|
| Airflex® 500 | A nonionic latex of ethylene vinyl acetate copolymer having an average particle size of 170 nm and a Tg of 5°C (41 °F) available from Air Products of Allentown, Pennsylvania. |
| | |
| Epson Stylus® Color 800 Printer | Ink jet printer available from Epson America, Inc. of Torrence, CA. |
| | |
| Epson Stylus® 800 Color Ink | Color ink jet cartridge containing cyan, magenta and yellow available from Epson America, Inc. of Torrence, CA under model number S020089. |
| | |
| Epson Stylus® 800 Black Ink | Black ink jet cartridge available from Epson America, Inc. of Torrence, CA under model number S020108. |
| | |
| MP1040™ | Particulate silica having a diameter of 100±30 nm available from Nissan Chemical Industries, Ltd. of Tokyo, Japan. |
| | |
| Imation™ Photograde Inkjet Paper | Paper sheets (8½ by 11) available from Imation Corp. of St. Paul, Minnesota. |
| | |
| PET | Polyethylene Terephthalate |
| | |
| PVDC | Polyvinylidenechloride |
| | |
| 3MSP3BAC1 | The cationic silane N-trimethoxysilylpropyl-N,N,N-tri-n-butyl ammonium chloride available from Gelest, Inc. of Tullytown, PA under catalog number SIT 8414.0. |
| 3MSEB3MAC1 | The cationic silane N-trimethoxysilylethyl benzyl-N,N,N-trimethyl ammonium chloride available from Gelest, Inc. of Tullytown, PA under catalog number SIS 6994.0. |

### Testing Procedures

### COLOR SATURATION TESTING PROTOCOL

Epson Stylus® Color 800™ ink is jetted from an Epson Stylus® Color 800™ printer onto the recording layer of the sample sheet in step patches ranging from 0 (no color) to 16 (full color saturation). Printed samples from midtone to full color patches (*i*.*e*., patches between 6 and 16) were selected for testing unless otherwise noted. Color saturation is measured with a Gretag™ spectrophotometer as the log of the ratio of the intensity of visible light given out by the bulb in the spectrophotometer over the intensity of visible light reflected by the printed sample. The color saturation is recorded.

### DROP SIZE TESTING PROTOCOL

Epson Stylus® Color 800™ ink is jetted from an Epson Stylus® Color 800™ printer onto the recording layer of an Imation™ Photograde Inkjet sample sheet for a midtone patch. Drop size of the jetted ink is viewed through a microscope, aimed perpendicular to the surface of the recording layer, giving a top view of the ink drop absorbed into the layer. The microscope is attached to a video camera and frame-grabber capable of permitting computer analysis and storage of the image. Computer analysis of the image yields drop size, with the average of approximately twenty five drops reported as the drop size for the sample.

### Standard Sample Construction

Into a beaker equipped with a magnetic stirrer was placed deionized water and MP1040™, in the amount set forth in Table One, to form a silica dispersion. The silica dispersion was stirred for 30 minutes. A silane coupling agent, of the type and in the amount set forth in Table One, was then optionally added to the silica dispersion and stirred overnight at approximately 25°C (77°F). Into the stirred silica dispersion was then added sodium sulfate, in the amount set forth in Table One, followed after 30 minutes of stirring by the addition of Airflex® 500, in the amount set forth in Table One, to form a final dispersion. The final dispersion was stirred for one to four hours prior to coating.

The stirred final dispersion was coated onto a PVDC primed PET sheet using a knife coater with a seven millimeter gap. The coated PET sheet was oven dried at 120°F (48.9°C) for seven minutes to form an ink jet recording sheet with a recording layer.

### Examples

### COMPARATIVE EXAMPLE C1

### EXAMPLE 1

### (Color Saturation and Drop Size)

### (Without Silane Coupling Agent)

Sample ink jet recording sheets having a recording layer were constructed in accordance with the Standard Sample Construction Procedure. The color saturation of the sample recording sheets was tested in accordance with the Color Saturation Testing Protocol. Drop size was tested in accordance with the Drop Size Testing Protocol. The results of the testing were recorded, and are set forth in Tables Two and Three, respectively.

As shown in Table Two, color saturation (density) and dot size (resolution) is generally improved for recording sheets having a recording layer containing the electrolyte sodium sulfate when compared to sheets with a recording layer containing no electrolyte, with the greatest improvement observed when conducting high saturation ink jet printing.

### COMPARATIVE EXAMPLES C2_{low}, C2_{med}, C2_{high} AND C3

### EXAMPLES 2A_{low}, 2A_{med}, 2A_{high}, 2B_{low}, 2B_{med}, 2B_{high} AND 3

### (Color Saturation and Drop Size)

### (Different Concentrations of Cationic Silane Coupling Agents)

Ink jet recording sheets having a recording layer containing different concentrations of a silane coupling agent were constructed in accordance with the Standard Sample Construction Procedure. The color saturation of the recording sheets was tested in accordance with the Color Saturation Testing Protocol. Drop size was also tested in accordance with the Drop Size Determination Protocol. The results of the testing were recorded, and are set forth in Tables Two and Three, respectively.

As shown in Table Two, color saturation (density) and dot size (resolution) is generally improved for recording sheets having a recording layer containing the electrolyte sodium sulfate when compared to sheets with a recording layer containing no electrolyte, with the greatest improvement observed when conducting high saturation ink jet printing.

## Claims

1. An ink jet recording sheet comprising:
(a) a substrate having first and second major surfaces, and
(b) a recording layer on at least one of the major surfaces of the substrate comprising at least:
(1) a binder,
(2) a pigment particle,
(3) an electrolyte, and
(4) a cationic organosilane coupling agent.

2. The inkjet recording sheet of claim 1 wherein the binder is a latex binder.

3. The ink jet recording sheet of any of claims 1 or 2 wherein the pigment particle is a silica pigment particle.

4. The ink jet recording sheet of any of claims 1-3 wherein the electrolyte is an acid or an inorganic salt.

5. The ink jet recording sheet of any of claims 1-4 wherein the cationic organosilane coupling agent has the structure:
R' L Si R"₃
wherein: (i) R' is a quaternary ammonium group, (ii) L is a single bond or divalent linking group, and (iii) each R" is independently an alkoxy group.

6. The ink jet recording sheet of any of claims 1-5 wherein the cationic organosilane coupling agent has the structure:
R'ₙ Si R"₍₄₋ₙ₎
wherein: (i) R' is R³₃N⁺L- where L is a single bond or divalent linking group, and each R³ is independently hydrogen, alkyl, aryl or alkaryl with at least two R³ being alkyl, aryl or alkaryl, (ii) each R" is independently an alkoxy group; and (iii) n is 1 or 2.

7. The ink jet recording sheet of any of claims 5 or 6 wherein (i) each R" is independently an alkoxy group containing 1 to 3 carbon atoms, and (ii) n is 1.

8. A method of making an ink jet recording sheet comprising:
(a) obtaining a substrate having first and second major surfaces,
(b) coating a layer of a recording composition on at least one of the major surfaces of the substrate wherein the recording composition is a dispersion containing at least (i) a binder, (ii) pigment particles, (iii) an electrolyte, and (iv) a cationic organosilane coupling agent, and
(c) drying the recording layer.

9. A method of using an inkjet recording sheet comprising:
(a) obtaining a substrate having a layer of a recording composition on at least one of the major surfaces of the substrate, wherein the recording composition is a dispersion comprising at least (i) a binder, (ii) pigment particles, (iii) an electrolyte, and (iv) a cationic organosilane coupling agent, and
(b) jetting inkjet printing ink upon the major surface of the substrate coated with the recording composition so as to produce an image upon the sheet.

## Patentansprüche

1. Flächengebilde zur Tintenstrahlaufnahme, umfassend:
(a) ein Substrat mit ersten und zweiten Hauptoberflächen, und
(b) eine Aufnahmeschicht auf mindestens einer der Hauptoberflächen des Substrats, mindestens umfassend:
(1) ein Bindemittel,
(2) ein Pigmentteilchen,
(3) einen Elektrolyt, und
(4) ein kationisches Organosilan-Kupplungsmittel.

2. Flächengebilde zur Tintenstrahlaufnahme nach Anspruch 1, wobei das Bindemittel ein Latexbindemittel ist.

3. Flächengebilde zur Tintenstrahlaufnahme nach einem der Ansprüche 1 oder 2, wobei das Pigmentteilchen ein Siliciumoxid-Pigmentteilchen ist.

4. Flächengebilde zur Tintenstrahlaufnahme nach einem der Ansprüche 1 bis 3, wobei der Elektrolyt eine Säure oder ein anorganisches Salz ist.

5. Flächengebilde zur Tintenstrahlaufnahme nach einem der Ansprüche 1 bis 4, wobei das kationische Organosilan-Kupplungsmittel die Struktur:
R' L Si R"₃
aufweist, wobei: (i) R' ein quartärer Ammoniumrest ist, (ii) L eine einfache Bindung oder ein divalenter verbindender Rest ist, und (iii) jedes R" unabhängig voneinander ein Alkoxyrest ist.

6. Flächengebilde zur Tintenstrahlaufnahme nach einem der Ansprüche 1 bis 5, wobei das kationische Organosilan-Kupplungsmittel die Struktur:
R'ₙ Si R"₍₄₋ₙ₎
aufweist, wobei: (i) R'R³₃N⁺L- ist, wobei L eine einfache Bindung oder ein divalenter verbindender Rest ist, und jedes R³ unabhängig voneinander ein Wasserstoffatom, Alkyl, Aryl oder Alkaryl ist, wobei mindestens zwei R³ Alkyl, Aryl oder Alkaryl sind, (ii) jedes R" unabhängig voneinander ein Alkoxyrest ist; und (üi) n 1 oder 2 ist.

7. Flächengebilde zur Tintenstrahlaufnahme nach einem der Ansprüche 5 oder 6, wobei (i) jedes R" unabhängig voneinander ein Alkoxyrest mit 1 bis 3 Kohlenstoffatomen ist, und (ii) n 1 ist.

8. Verfahren zum Herstellen eines Flächengebildes zur Tintenstrahlaufnahme, umfassend:
(a) Erlangen eines Substrats mit ersten und zweiten Hauptoberflächen,
(b) Auftragen einer Schicht einer Aufnahmezusammensetzung auf mindestens eine der Hauptoberflächen des Substrats, wobei die Aufnahmezusammensetzung eine Dispersion mit mindestens (i) einem Bindemittel, (ii) Pigmentteilchen, (iii) einem Elektrolyt, und (iv) einem kationischen Organosilan-Kupplungsmittel ist, und
(c) Trocknen der Aufnahmeschicht.

9. Verfahren zur Verwendung eines Flächengebildes zur Tintenstrahlaufnahme, umfassend:
(a) Erlangen eines Substrats mit einer Schicht einer Aufnahmezusammensetzung auf mindestens einer der Hauptoberflächen des Substrats, wobei die Aufnahmezusammensetzung eine Dispersion umfassend mindestens (i) ein Bindemittel, (ii) Pigmentteilchen, (iii) einen Elektrolyt, und (iv) ein kationisches Organosilan-Kupplungsmittel ist, und
(b) Aufbringen der Tintenstrahldrucktinte auf die mit der Aufnahmezusammensetzung beschichtete Hauptoberfläche des Substrats, so dass ein Bild auf dem Flächengebilde hergestellt wird.

## Revendications

1. Feuille d'enregistrement pour jet d'encre comprenant :
(a) un substrat ayant une première et une seconde surfaces majeures, et
(b) une couche d'enregistrement sur au moins l'une des surfaces majeures du substrat, comprenant au moins :
(1) un liant,
(2) une particule de pigment,
(3) un électrolyte, et
(4) un agent de couplage d'organosilane cationique.

2. Feuille d'enregistrement pour jet d'encre selon la revendication 1, dans laquelle le liant est un liant de latex.

3. Feuille d'enregistrement pour jet d'encre selon l'une quelconque des revendications 1 ou 2, dans laquelle la particule de pigment est une particule de pigment de silice.

4. Feuille d'enregistrement pour jet d'encre selon l'une quelconque des revendications 1 à 3, dans laquelle l'électrolyte est un acide ou un sel inorganique.

5. Feuille d'enregistrement pour jet d'encre selon l'une quelconque des revendications 1 à 4, dans laquelle l'agent de couplage d'organosilane cationique a la structure :
R'LSiR''₃
dans laquelle : (i) R' représente un groupe d'ammonium quaternaire, (ii) L représente une liaison unique ou un groupe de liaison divalent, et (iii) chaque groupe R'' représente indépendamment un groupe alcoxy.

6. Feuille d'enregistrement pour jet d'encre selon l'une quelconque des revendications 1 à 5, dans laquelle l'agent de couplage d'organosilane cationique a la structure :
R'ₙSiR''₍₄₋ₙ₎
dans laquelle : (i) R' représente le groupe R³₃N⁺L-, où L représente une liaison unique ou un groupe de liaison divalent, et chaque groupe R³ représente indépendamment un atome d'hydrogène, un groupe alkyle, aryle ou alkaryle avec au moins deux groupes R³ représentant un groupe alkyle, aryle ou alkaryle, (ii) chaque groupe R'' représente indépendamment un groupe alcoxy ; et (iii) n est égal à 1 ou 2.

7. Feuille d'enregistrement pour jet d'encre selon l'une quelconque des revendications 5 ou 6, dans laquelle (i) chaque groupe R'' représente indépendamment un groupe alcoxy contenant 1 à 3 atomes de carbone, et (ii) n est égal à 1.

8. Procédé de préparation d'une feuille d'enregistrement pour jet d'encre comprenant les étapes consistant à :
(a) obtenir un substrat ayant une première et une seconde surfaces majeures,
(b) revêtir une couche d'une composition d'enregistrement sur au moins l'une des surfaces majeures du substrat, la composition d'enregistrement étant une dispersion contenant au moins (i) un liant, (ii) des particules de pigment, (iii) un électrolyte, et (iv) un agent de couplage d'organosilane cationique, et
(c) sécher la couche d'enregistrement.

9. Procédé d'utilisation d'une feuille d'enregistrement pour jet d'encre comprenant les étapes consistant à :
(a) obtenir un substrat ayant une couche d'une composition d'enregistrement sur au moins l'une des surfaces majeures du substrat, la composition d'enregistrement étant une dispersion comprenant au moins (i) un liant, (ii) des particules de pigment, (iii) un électrolyte, et (iv) un agent de couplage d'organosilane cationique, et
(b) projeter l'encre d'impression par jet d'encre sur la surface majeure du substrat revêtu de la composition d'enregistrement afin de produire une image sur la feuille.
